# EUROPEAN PATENT SPECIFICATION

(11) **EP 1 234 065 B1**
(45) Date of publication and mention of the grant of the patent: **22.03.2006**
(21) Application number: 00973247.0
(22) Date of filing: 07.11.2000
(51) Int. Cl.: D01F 6/06

(54) **POLYPROPYLENE FIBER AND PREPARATION THEREOF**
POLYPROPYLENFASER UND VERFAHREN ZU SEINER HERSTELLUNG
FIBRE DE POLYPROPYLENE ET SA PREPARATION

(30) Priority: 10.11.1999 KR 9949610; 16.03.2000 KR 2000013319
(43) Date of publication of application: 28.08.2002
(73) Proprietor: Park, Pyung Yul, Kimchom-si, Kyongsangduk-do 740-755 (KR)
(72) Inventor: PARK, Pyung, Yul, Kimchom-si, Kyongsangduk-do 740-755 (KR); CHEY, Won, Jun, Talso-gu, Taegu 704-350 (KR)
(74) Representative: Texier, Christian
(86) International application number: PCT/KR2000/001270
(87) International publication number: WO 2001/034884

(56) References cited:
- EP-A- 0 518 316
- JP-A- 5 009 810
- JP-A- 10 195 714

## Description

### BACKGROUND OF THE INVENTION

### 1. Field of the invention

The present invention relates, in general, to a polypropylene fiber and, more particularly, to a polypropylene fiber which is useful as a material for non-woven fabrics, thereby allowing the non-woven fabrics to be smooth and excellent in strength and providing workability and physical properties for the non-woven fabrics during after-processes. Also, the present invention is concerned with a method for preparing such fibers.

### 2. Description of the Prior Art

In order that staple fibers are prepared from polyolefin polymers, they have to undergo a series of processes: the polyolefin polymers are generally compounded with some amount of additives and the resulting mixtures are melt-extruded in ordinary commercial processes to give fibers, which are crimped and cut into predetermined lengths.

When being applied for the making of non-woven fabrics, polyolefin staples are typically processed in a carding machine to give non-woven webs which are then thermally bonded.

For thermal bonding, a pair of calender rollers, ultrasonification, or hot air is usually used.

Particularly as for polypropylene filaments or staples, they are arranged after opening and carding processes, and bridged to afford webs. These webs are thermally bonded with the aid of a calender roller with diamond or delta type patterns to produce non-woven fabrics which are industrially useful in various fields. Alternatively, hot air may be utilized instead of calender rollers. In this case, after being allowed to undergo a carding process, webs are bonded to give non-woven fabrics by means of hot air which is circulated in a porous drum.

Polypropylene non-woven fabrics find numerous applications in the disposable diaper, diaper for patients suffering from urinary incontinence, hygienic band, mask, and medical fabric industries. Although not demanding strength as high as that of woven fabrics, the non-woven fabrics used in these purposes have to be soft and satisfy the requirement of safety to skin because they are in direct contact with the skin.

The strength of non-woven fabrics varies depending on their preparation processes as well as on physical properties of material fibers.

With the aim of improving productivity, non-woven fabric producing manufacturers generally try to make high production speed. The high production speed, however, demands more excellent physical properties for the fibers for non-woven fabrics.

Prior art document EP-0518316 discloses a stretched molded article of ultra-high-molecular-weight polypropylene having an intrinsic viscosity [η] of at least 4 dl/g, which has a degree of orientation of not less than 0.930 when obtained as a degree of orientation by an X-ray diffraction half-width, two or more of peak positions (melting points) within the temperature region of not lower than 180°C when measured by a differential scanning calorimeter, and an amount of output energy of not less than 1 kgfm/g after 10-time repetition under a load of 50% of the breaking strength. EP-0518316 also discloses a process for the preparation of a stretched molded article of ultra-high- molecular-weight polypropylene having a large amount of output energy comprising the steps of :
(i) extruding through a molding die or a nozzle an ultra-high-molecular-weight polypropylene composition composed of 15 - 80 parts by weight of ultra-high-molecular-weight polypropylene having an intrinsic viscosity [η] of at least 4 dl/g and 85 - 20 parts by weight of a diluent at a temperature at which the composition is flowable,
(ii) taking up the extrudate in a draft radio of at least 3 times and then recrystallizing the ultra-high-molecular-weight polypropylene contained in the extrude during or after the take-up procedure to form an unstretched orientation product, and
(iii) stetching the unstretched orientation product at least once in a draw ratio of at least 3 times at a temperature of not lower than 90° C.

### SUMMARY OF THE INVENTION

Leading to the present invention, the intensive and thorough research on polypropylene yarns or staples suitable for non-woven fabrics, repeated by the present inventors aiming to overcome the above problems encountered in prior arts, resulted in the finding thatisotactic polypropylene homopolymers, which are found to have two endothermic peaks as measured by a differential scanning calorimeter (DSC), allow the production of novel fibers, which have been not yet reported in the arts, and guarantee the excellent strength and softness of the non-woven fabrics prepared from the fibers. In addition, the fibers of such a structure were found to be obtained by controlling melting indexes and polydispersity indexes in each process step through the total procedure.

Therefore, it is an object of the present invention to provide polypropylene fibers for non-woven fabrics, which can be applied to high-speed carding machines and guarantee the excellent strength and softness of the non-woven fabrics after thermal bonding.

It is another object of the present invention to provide a method for preparing such polypropylene fibers.

It is a further object of the present invention to provide a non-woven fabric prepared from such polypropylene fibers.

In accordance with an embodiment of the present invention, there is provided a polypropylene fiber, which is obtained from an isotactic polypropylene homopolymer with an isotactic index of 90 to 99 % through melt-spinning or through drawing after melt-spinning, and shows two differential scanning calorimeter (DSC) endothermic peaks between 155 and 170 °C, said fiber having a melt index (MI_{c}) of 16.5 to 80.0 and a polydispersity index (PI_{c}) of 2.1 to 5.7.

In accordance with another embodiment of the present invention, there is provided a method for preparing polypropylene fibers, comprising the steps of: (a) melting in an extruder an isotactic polypropylene homopolymer with an isotactic index of 90-99 %, a melting index (MIₐ) of 10.0-40.0, preferably 10.0-25.0 and a polydispersity index ( PIₐ) of 2.5-6.0, preferably 2.8-5.0 and more preferably 3.5-4.3 to give a molten polymer which has a melt index (MI_{b}) with the ratio of MI_{b}/MIₐ ranging from 1.01 to 1.50 and a polydispersity index (PI_{b}) narrower by 10 % or less than the PI_{a;} (b) spinning the molten polymer and controlling the quenching condition after the spinning to produce fibers with a melting index (MI_{c}) of 16.5-80.0 and a polydispersity index (PI_{c}) narrower by 20% or less than the PIₐ, the ratio of MI_{c}/MIₐ ranging from 1.65 to 7.50; and (c) optionally drawing the fibers.

### BRIEF DESCRIPTION OF THE DRAWINGS

The above and other objects, features and other advantages of the present invention will be more clearly understood from the following detailed description taken in conjunction with the accompanying drawings, in which:
Fig. 1 is a DSC endothermic curve in which two endothermic peaks apparently appear in a polypropylene homopolymer fiber of the present invention as measured by a DSC;
Fig. 2 is a DSC endothermic curve in which two endothermic peaks apparently appear with the secondary peak being in a shoulder form of the primary peak; and
Fig. 3 is a DSC endothermic curve in which only one DSC endothermic peak appears in a conventional polypropylene homopolymer fiber.

### DETAILED DESCRIPTION OF THE INVENTION

The present invention pertains to polypropylene fibers which are prepared from polypropylene homopolymers with an isotactic index of 90 to 99% by melt-spinning or by melt-spinning and drawing and have two differential scanning calorimeter (DSC) endothermic peaks in the range from 155 to 170 °C. Preferably, the polypropylene fibers of the present invention show a primary endothermic peak at 160±3 °C and a secondary endothermic peak at 165±3 °C.

Where non-woven fabrics are prepared from the polypropylene fibers of the present invention by thermal bonding, the above physical properties allow the non-woven fabrics to be smooth with excellent strength. This advantage is believed to result from the fact that, while the fibers thermally fused due to the heat or the heat and the pressure between rolls are solidified again, rapid recrystallization occurs in the regions which are high in melting points.

Useful as materials to prepare the fibers of the present invention are polypropylene homopolymers with an isotactic index of 90 to 99 %.

The polypropylene fibers of the present invention have a melt index (MI_{c}) of 16.5-80.0, which is preferably 1.65-7.50 times as large as that (MIₐ) of the material isotactic polypropylene.

The polypropylene fibers of the present invention range, in polydispersity index (PI_{c}), from 2.1 to 5.7 and, preferably from 3.5 to 4.3 with a value being narrower by 20 % than the PIₐ of the material isotactic polypropylene.

A preferable fineness that the polypropylene fibers of the present invention have falls in the range of 1.0 to 80.0 deniers.

As for the isotactic polypropylene used in the present invention, it preferably ranges, in melt index (MIₐ), from 10 to 40 and, in polydispersity index (PIₐ), from 2.5 to 6.0.

When the polypropylene is melted in an extruder, a stabilizer or an antioxidant is preferably formulated at an amount of 0.03 to 2.0 wt%, preferably 0.03 to 0.7 wt% and more preferably 0.03 to 0.4 wt%.

In addition to stabilizers or antioxidants, ordinary additives in the art, such as a deoxidant agent, a colorant, metal carboxylates, etc., may be used for the preparation of the fibers of the present invention. The metal carboxylate available in the present invention is selected from the group consisting of nickel salts of 2-ethyl hexanoic acid, caprylic acid, decanoic acid, and dodecanoic acid, Fe, Co, Ca and Ba salts of 2-ethyl hexanoic acid, and combinations thereof. As the deoxidant agent or the colorant, calcium stearate, which is usually used to prepare polypropylene homopolymers in petrochemical plants, may be selected. A variety of additives available in the present invention may be referred to European patent No. 279,511.

The isotactic polypropylene useful in the present invention, as previously mentioned, preferably has a melt index (MIₐ) of 10 to 40. For example, when the MIₐ is below 10, an increase occurs in the spinneret pressure upon spinning, giving rise to a decrease in productivity. A high heat is required for the melt-spinning of such polypropylene, resulting in an increase in energy consumption. In addition, the fibers obtained under such a high heat show increased tenacity, so that they are not suitable for the non-woven fabric uses which require smoothness. On the other hand, when the isotactic polypropylene has an MIₐ of greater than 40, the resulting fibers are not suitable for non-woven fabrics in terms of strength. Further, incompletion frequently occurs in the fulfillment of quenching after the spinning, leading to fusion between neighboring fibers.

It should be noted that the fibers of the present invention include those which are obtained through melting, spinning, solidifying and taking-up processes as well as those which are obtained through a drawing process after melting and spinning processes and necessarily have undergone the processes of crimping, thermal fixing and cutting into staples. The fibers which experience melt-spinning are almost identical to those which further experience drawing in MI, PI and DSC endothermic peak.

In an embodiment of the preparation of polypropylene filaments or staples according to the present invention, the material polymer is melted in an extruder to give a molten polymer which has a melt index (MI_{b}) with the ratio of MI_{b}/MIₐ ranging from 1.01 to 1.50 and a polydispersity index (PI_{b}) being narrower by 10 % than PIₐ and more preferably by 5 %. A preferable PI_{b} falls in the range of 2.4 to 5.0.

For example, if MI_{b} exceeds 1.5 times of MIₐ, the molecular chain of the polypropylene is so cleaved that its inherent strength cannot be maintained. In addition, such cleavage leads to an insufficient viscosity for the molecular chains to orient at the nozzle, as well as cannot maintain a pressure suitable for spinning. Further, the fibers obtained are poor in strength, so that the non-woven fabrics prepared from the fibers feel harsh to the touch. In result, the productivity becomes poor. An MI change as large as or larger than 1 % naturally occurs in the polypropylene upon extrusion. When MI_{b} is changed to less than 1.01 times of MIₐ, serious difficulty is found in the preparation process of fibers. Particularly, a high viscosity at the nozzle appears to increase the pressure of the nozzle, making the spinning process very unstable. Accordingly, the production yield is lowered with a serious deviation in fiber quality.

By controlling the quenching condition after the spinning, the polymer which has undergone an MI change in the extruding process, is allowed to be secondarily changed in MI. The MI change at a quenching step is determined depending on the temperature of the delayed quenched region, the atmosphere, the temperature, speed and quantity of quenching air. U.S. Pat. No. 4,193,961 describes the use of delay quenching and quenching air, which may also be referred to other documents, for example, M. Ahmed "Polypropylene Fibers-Science and Technology" sponsored by Society of Plastics Engineers, Inc.

In accordance with the preparation of the present invention, the fibers which experience the quenching step are preferably controlled to have a melt index (MI_{c}) 1.65-7.50 times as large as the melt index (MIₐ) of the material polymer and a polydispersity index (PI_{c}) narrower by 20 % or less than that (PIₐ) of the material polymer (that is, amounts to 0.80x,PIₐ or wider). The fibers preferably range, in PI_{c}, from 2.1 to 5.7, more preferably from 2.3 to 4.5 and most preferably from 3.0 to 4.0.

When the MI_{c} is over the above range, the strength of the grey yarns is deteriorated. The making of non-woven fabrics from the grey yarns suffers from poor workability because the non-woven fabrics are apt to be contaminated with card clothing and partially melted on the calender roll. In detail, if the MI_{c} deviates from the upper limit, the yarn has a too greatly decreased molecular weight and the quenching effect after the spinning from a nozzle is decreased to generate fusion between yarns. Where the yarns are used to make non-woven fabrics after being forcibly prepared in spite of the above conditions, much powder is generated from the poor yarns in an opening and a carding process, having a negative influence on the making process. In addition, heat-vulnerable portions of the poor yarns are melt out upon calendering, making dirty the surface of the calender roll which plays a role in the final thermal bonding of the non-woven fabrics.

On the other hand, if the MI_{c} is beyond the lower limit, the strength of the grey yarn is improved, but it is difficult for such grey yarns to improve the thermal bonding index (hereinafter referred to as "TBI") to a desired extent. That is, the non-woven fabrics obtained show low TBI and feel harsh to the touch. Although the strength or TBI of the non-woven fabrics can be improved by increasing the temperature of the calender roll or the thermal bonding area, the non-woven fabrics still remain harsh.

Upon the making of non-woven fabrics, their machine direction orientation and cross direction strengths vary depending on the kinds and arrangements of carding machines. Differences may be found in the machine direction and cross direction strengths of the non-woven fabrics which have passed through carding machines if these machines are manufactured by different manufacturers. Even in the carding machines manufactured by the same manufacturers, the non-woven fabrics show different physical properties in dependence on the shape and material of carding clothing and the presence of random rolls. In addition, the non-woven fabrics are different in plan weight, depending on the requirements for the after-process. The measured strength values of the non-woven fabrics represent simple tenacity and their units are characteristically different from one company to another. Therefore, since there may occur a case in that superiority cannot be discriminated therebetween, the simple tenacity is unsuitable to determine whether the physical properties of the non-woven fabrics are improved. However, the structure and inherent physical properties of the yarn or staple can be compared as to the influence on the non-woven fabrics by reference to the bonding indexes of the non-woven fabrics prepared although a difference may exist in kinds or arrangements of the carding machines.

In accurately determining the influence of the physical properties of yarns or staples on the non-woven fabrics thereof, therefore, the concept of TBI is recognized as very proper. A detail of TBI is described in an article concerning Polypropylene Fibres and Textiles, reported in the Fourth International Conference held by The Plastics and Rubber Institute. Indeed, TBI is introduced in the present invention as the most valuable parameter to comparatively determine the influence of the physical properties of yarns or staples on the non-woven fabrics.

Of the fibers of the present invention, the non-woven fabrics can be made which are 2.0 or higher in TBI with good softness.

A better understanding of the present invention may be obtained in light of the following examples which are set forth to illustrate, but are not to be construed to limit the present invention.

In the following Examples, fibers and non-woven fabrics suggested in the present invention were analyzed for physical properties.

DSC endothermic Peaks: fiber samples were sufficiently washed to remove oiling agents. After being dried for 30 min in the air, the samples were vacuum-dried for 1 hour in a decicater and cut into a length of 2-4 mm. The cut samples of 5mg were put on a measuring pan which was then subjected to thermal analysis using the Perkin Elmer 7 series Thermal Analysis System in which the temperature was elevated at a rate of 5 °C/min from 30 °C to 190 °C, so as to obtain endothermic curves. Other conditions of this measurement were accorded with ASTM 3418-82 method. Conventional polypropylene homopolymer fibers showed single endothermic peaks while the fibers of the present invention have double endothermic peaks, as exhibited in the accompanying drawings. Fig. 1 shows two apparent DSC endothermic peaks of the fiber according to the present invention and Fig. 2 shows that a secondary DSC endothermic peak appears in a shoulder form of a primary DSC endothermic peak. Fig. 3 is an endothermic curve showing that only one DSC endothermic peak appears in a conventional fiber.

Denier of Yarn and Staple: measured using Vibroskop, manufactured by Lenzing.

Strength and Elongation of Yarn and Staple: measured using Vibrodyn, manufactured by Lenzing, according to ASTM D 638.

Melt Index (MI): measured using Model MP 993 of Tinius Olsen, according to ASTM D 1238. For the measurement of MI, the fiber samples were washed with copious water, centrifuged, dried at 105 °C for 15 min in an oven and cut into 1 cm.

Polydispersity Index (PI): using Model RMS-800(Disk; parallel plate) of Rheometrics, U.S.A., G_{c} was measured at 200 °C at a shear rate of 0.1-100 under a 10% strain condition and substituted into the following equation. $PI = \frac{{10}^{6}}{{G}_{c}}$
wherein G_{c} is a modulus of a point at which a storage modulus (G') and a loss modulus (G") are crossed with each other at two to six frequencies in a frequency range of 5-250 Hz. When there occurred no cross points, G_{c} was determined by extrapolation.

Isotactic Index (I.I.): a polypropylene homopolymer sample was cut into a length of 5 mm, washed with water, and dried at 105 °C for 1 hour in an oven. After taking about 5g and then being accurately weighed, a portion of the dried sample was boiled for about 5 hours in heptane for extraction. After completion of the extraction, the sample was sufficiently washed with water, dried at 105 °C for 1 hour in an oven and then weighed. The weights measured before and after the extraction were substituted in the following equation to yield the isotactic index.$Isotactic Index ( % ) = \frac{Weight After Extraction}{Weight Before Extraction} \times 100$

Thermal Bonding Index (TBI) of Non-Woven Fabric: calculated according to the following mathematical equation: $TBI = {( MD \times CD )}^{1 / 2} \times \frac{20}{Plan Weight}$
wherein, MD is a machine direction strength (kg/50 mm), CD is a cross direction strength (kg/50 mm), and plan weight is a weight per area of a non-woven fabric.

Strength of Non-Woven Fabric: samples with a dimension of 50 mm width and 140 mm length were measured at a tensile speed of 100 mm/min using an instron.

Softness : the feeling to the touch was graded: 1 very harsh; 2 harsh; 3 ordinary; 4 soft; 5 very soft.

### EXAMPLES 1 TO 7 AND COMPARATIVE EXAMPLES 1 TO 7

Isotactic polypropylene homopolymers with an isotatic index of 97% and MI as indicated in Table 1, below, containing an antioxidant and stabilizer at an amount of 0.09 wt%, were melt-spun at an extruder temperature from 250 to 290 °C while the heating in the range from the extruder to the nozzle was controlled in the range of 285-310 °C by means of a heating medium to allow the melt to have MI_{b} as indicated in Table 1, below. For the comparison of MI between the raw material and the melt before the nozzle, a bypass was set to take the samples while a minimization was provided to the pressure just before a gear pump which served to constantly feed the melt into the nozzle.

Next, the melt was extruded at a spinning rate of 1,500 m/min through a spinneret, passed through a heat reserving zone for delayed quenching and then quenched to afford primary yarns of 2.4 deniers, which had Mic, PIc and DSC endothermic peaks as shown in Table 1.

The primary yarns thus obtained were collected in a bundle and drawn at a drawing ratio of 1.5 times while being crimped in a crimper, following cutting them to staples 40 mm long.

Given in Table 2 are MI, PI, fiber strength, number of crimps and DSC endothermic peaks of the staples obtained.

In order to prepare non-woven fabrics, the staples were applied to the carding machines according to manufacturers. The upper roll used for the preparation of non-woven fabrics was of a diamond type with a sealing area amounting to 22 % while the calender roll performed its function at 147 °C with a pressure of 95 kg/cm.

The non-woven fabrics obtained are described concerning plan weight, strength of machine direction and cross direction, TBI and softness in Table 3, below.

**TABLE 2**

| Nos. of | | Ml_{c} | | Pl_{c} | Strength of Fiber (g/d) | CrimpNos. | DSC EndothermicPeaks of staple (°C) | |
|---|---|---|---|---|---|---|---|---|
| Exmpl. | Fiber Spun | Staple drawn After spin | Fiber spun | Staple drawn After spin | | | 1 | 2 |
| 1 | 52.0 | 51.0 | 3.8 | 3.7 | 1.9 | 7.7 | 159.4 | 164.2 |
| 2 | 56.0 | 55.0 | 2.9 | 2.8 | 2.2 | 6.2 | 160.1 | 164.5 |
| 3 | 57.0 | 57.6 | 4.5 | 4.5 | 2.3 | 6.4 | 159.7 | 165.8 |
| 4 | 36.5 | 36.9 | 4.9 | 5.0 | 1.9 | 6.4 | 158.9 | 165.1 |
| 5 | 45.0 | 44.0 | 3.6 | 3.8 | 2.4 | 7.2 | 160.2 | 164.1 |
| 6 | 46.0 | 47.3 | 3.5 | 3.4 | 2.2 | 6.2 | 159.8 | 165.8 |
| 7 | 31.2 | 33.0 | 4.9 | 4.8 | 2.6 | 5.9 | 159.9 | 163.7 |
| C.1 | 24.3 | 24.3 | 2.2 | 2.3 | 2.2 | 7.5 | 160.1 | - |
| C.2 | 106.5 | 104.2 | 6.5 | 6.5 | 1.7 | 7.6 | 160.2 | |
| C.3 | 32.3 | 33.6 | 5.1 | 5.2 | 2.2 | 6.5 | 160.3 | - |
| C.4 | 80.2 | 81.2 | 4.7 | 4.9 | 1.9 | 8.1 | 160.4 | - |
| C.5 | 28.0 | 29.3 | 4.2 | 4.3 | 2.1 | 6.9 | 160.1 | - |
| C.6 | 39.6 | 41.2 | 10.2 | 10.3 | 1.6 | 7.2 | 160.2 | - |
| C.7 | 201.0 | 197.0 | 5.1 | 5.2 | 1.7 | 6.5 | 160.1 | - |

**TABLE 3**

| Nos. of Exmpl. | Carding | | | Strength (kg/5cm) | | TBI | Softness | Notes |
|---|---|---|---|---|---|---|---|---|
| | Machines | Speed (m/min) | Plan Wt.(g/m²) | MD | CD | | | |
| 1 | THIBEAU | 180 | 21.0 | 5.3 | 1.4 | 2.6 | 5 | - |
| 2 | SPINNBAU | 175 | 19.0 | 5.2 | 1.2 | 2.6 | 4 | - |
| 3 | SPINNBAU | 100 | 19.5 | 7.2 | 2.6 | 4.4 | 5 | - |
| 4 | SPINNBAU | 210 | 17.8 | 6.2 | 1.5 | 3.4 | 4 | - |
| 5 | HERGETH | 95 | 20.1 | 4.9 | 1.8 | 3.0 | 5 | - |
| 6 | HERGETH | 95 | 22.1 | 6.8 | 1.8 | 3.2 | 4 | - |
| 7 | HERGETH | 180 | 20.3 | 3.9 | 1.4 | 2.3 | 4 | - |
| C.1 | SPINNBAU | 100 | 20.2 | 3.2 | 0.9 | 1.7 | 1 | Harsh |
| C.2 | HERGETH | 150 | 21.0 | 3.5 | 0.8 | 1.6 | 3 | TBI decrese |
| C.3 | SPINNBAU | 150 | 20.3 | 3.4 | 0.9 | 1.7 | 1 | TBI decrese |
| C.4 | SPINNBAU | 160 | 20.4 | 3.5 | 1.0 | 1.8 | 2 | TBI decrese |
| C.5 | SPINNBAU | 100 | 19.8 | 3.8 | 0.9 | 1.9 | 2 | Harsh |
| C.6 | SPINNBAU | 105 | 18.9 | 3.9 | 0.8 | 1.9 | 2 | Harsh |
| C.7 | SPINNBAU | 90 | 19.5 | 3.8 | 0.9 | 1.9 | 3 | Difficult, much NEP |

As apparent from the above examples, the non-woven fabrics, which are prepared by thermally bonding the isotactic polypropylene homopolymer fibers having two DSC endothermic peaks in accordance with the present invention, show excellent strength in addition to being soft. Also, the non-woven fabrics can be produced in high speed carding machines. Consequently, the present invention allows the production of high quality non-woven fabrics with a high yield.

The present invention has been described in an illustrative manner, and it is to be understood that the terminology used is intended to be in the nature of description rather than of limitation. Many modifications and variations of the present invention are possible in light of the above teachings. Therefore, it is to be understood that within the scope of the appended claims, the invention may be practiced otherwise than as specifically described.

## Claims

1. A polypropylene fiber, which is obtained from an isotactic polypropylene homopolymer with an isotactic index of 90 to 99 % through melt-spinning or through drawing after melt-spinning, and shows two differential scanning calorimeter (DSC) endothermic peaks between 155 and 170 C°, said fiber having a melt index (MI_{c}) of 16.5 to 80.0 and a polydispersity index (PI_{c}) of 2.1 to 5.7.

2. The polypropylene fiber as set forth in claim 1, wherein the two differential scanning calorimeter. (DSC) endothermic peaks are composed of a primary endothermic peak appearing at 160±3 °C and a secondary endothermic peak appearing at 165±3 °C.

3. The polypropylene fiber as set forth in claim 1, wherein the fiber has a melt index (MI_{c}) of 16.5-80.0.

4. The polypropylene fiber as set forth in claim 1, wherein the fiber has a polydispersity index (PI_{c}) of 2.1-5.7.

5. The polypropylene fiber as set forth in claim 1, wherein the fiber has a fineness of 1.0-80.0 deniers per filament.

6. The polypropylene fiber as set forth in claim 4, wherein the fiber has the PI_{c} of 2.3-4.5.

7. The polypropylene fiber as set forth in claim 1, further comprising a stabilizer and/or an antioxidant at an amount of 0.03 to 2.0 wt%.

8. The polypropylene fiber as set forth in claim 7, wherein the stabilizer and/or an antioxidant is contained an amount of 0.03 to 0.7 wt%.

9. The polypropylene fiber as set forth in claim 8, wherein the stabilizer and/or an antioxidant is contained at an amount of 0.03 to 0.4 wt%.

10. A method for preparing polypropylene fibers, comprising the steps of:
(a) melting in an extruder an isotactic polypropylene homopolymer with an isotactic index of 90-99 %, a melting index (MIₐ) of 10.0-40.0 and a polydispersity index (PIₐ) of 2.5-6.0 to give a molten polymer which has a melt index (MI_{b}) with the ratio of MI_{b}/MIₐ ranging from 1.01 to 1.50 and a polydispersity index (PI_{b}) narrower by 10 % or less than the PIₐ;
(b) spinning the molten polymer and controlling the quenching condition after the spinning to produce fibers with a melting index (MI_{c}) of 16.5-80.0 and a polydispersity index (PI_{c}) narrower by 20 % or less than the PIₐ, the ratio of MI_{c}/MIₐ ranging from 1.65 to 7.50; and
(c) optionally drawing the fibers.

11. A method as set forth in claim 10, wherein the polypropylene homopolymer contains a stabilizer and/or an antioxidant at an amount of 0.03-2.0 wt% in the step (a).

12. A method as set forth in claim 10, wherein the MIₐ ranges from 10 to 30.

13. A method as set forth in claim 10, wherein the PIₐ ranges from 2.8 to 5.0.

14. A method as set forth in claim 13, wherein the PIₐ ranges from 3.5 to 4.3.

15. A method as set forth in claim 10, wherein the fibers range, in fineness, from 1.0 to 80.0 deniers per filament.

16. A method as set forth in claim 10, wherein the MI_{b} ranges 10.1-41.0.

17. A method as set forth in claim 10, wherein the fiber has the PI_{c} of 2.1-5.7.

18. A method as set forth in claim 17, wherein the fiber has the PI_{c} of 2.3-4.5.

## Revendications

1. Fibre de polypropylène, qui est obtenue à partir d'un homopolymère de polypropylène isotactique avec un indice d'isotacticité de 90 à 99 % par filage par fusion ou par étirage après filage par fusion, et présente deux pics endothermiques par analyse au calorimètre différentiel à balayage (DSC) entre 155 et 170 °C, ladite fibre ayant un indice de matière fondue (MI_{c}) de 16,5 à 80,0 et un indice de polydispersité (PI_{c}) de 2,1 à 5,7.

2. Fibre de polypropylène selon la revendication 1, dans laquelle les deux pics endothermiques par analyse au calorimètre différentiel à balayage (DSC) sont composés d'un pic endothermique primaire apparaissant à 160 ± 3 °C et un pic endothermique secondaire apparaissant à 165 ± 3 °C.

3. Fibre de polypropylène selon la revendication 1, dans laquelle la fibre a un indice de matière fondue (MI_{c}) de 16,5-80,0.

4. Fibre de polypropylène selon la revendication 1, dans laquelle la fibre a un indice de polydispersité (PI_{c}) de 2,1-5,7.

5. Fibre de polypropylène selon la revendication 1, dans laquelle la fibre a une finesse de 1,0-80,0 denier par filament.

6. Fibre de polypropylène selon la revendication 4, dans laquelle la fibre a un PI_{c} de 2,3-4,5.

7. Fibre de polypropylène selon la revendication 1, comprenant en outre un stabilisateur et/ou un anti-oxydant en une quantité de 0,03 à 2,0 % en poids.

8. Fibre de polypropylène selon la revendication 7, dans laquelle le stabilisateur et/ou l'anti-oxydant est contenu en une quantité de 0,03 à 0,7 % en poids.

9. Fibre de polypropylène selon la revendication 8, dans laquelle le stabilisateur et/ou l'anti-oxydant est contenu en une quantité de 0,03 à 0,4 % en poids.

10. Procédé de préparation de fibres de polypropylène, comprenant les étapes de :
(a) fusion dans une extrudeuse d'un homopolymère de polypropylène isotactique avec un indice d'isotacticité de 90-99 %, un indice de matière fondue (MIₐ) de 10,0-40,0 et un indice de polydispersité (PIₐ) de 2,5-6,0 pour donner un polymère fondu qui a un indice de matière fondue (MI_{b}) avec le rapport MI_{b/}MIₐ situé dans la gamme de 1,01 à 1,50 et un indice de polydispersité (PI_{b}) plus étroit de 10 % ou moins par rapport à PIₐ ;
(b) filage du polymère fondu et contrôle des conditions de trempe après le filage pour produire des fibres avec un indice de matière fondue (MI_{c}) de 16,5-80,0 et un indice de polydispersité (PI_{c}) plus étroit de 20 % ou moins par rapport à PIₐ, le rapport de MI_{c/}MIₐ étant dans la gamme de 1,65 à 7,50 ; et
(c) éventuellement étirage des fibres.

11. Procédé selon la revendication 10, dans lequel l'homopolymère de polypropylène contient un stabilisateur et/ou un anti-oxydant en une quantité de 0,03-2,0 % en poids à l'étape (a)

12. Procédé selon la revendication 10, dans lequel MIₐ est dans la gamme de 10 à 30.

13. Procédé selon la revendication 10, dans lequel PIₐ est dans la gamme de 2,8 à 5,0.

14. Procédé selon la revendication 13, dans lequel PIₐ est dans la gamme de 3,5 à 4,3.

15. Procédé selon la revendication 10, dans lequel les fibres sont dans la gamme de finesse de 1,0 à 80,0 denier par filament.

16. Procédé selon la revendication 10, dans lequel MI_{b} est dans la gamme de 10,1 à 41,0.

17. Procédé selon la revendication 10, dans lequel la fibre a un PI_{c} de 2,1-5,7.

18. Procédé selon la revendication 17, dans lequel la fibre a un PI_{c} de 2,3-4,5.S

## Patentansprüche

1. Polypropylen-Faser, die durch Schmelzspinnen oder durch Strecken nach Schmelzspinnen aus einem isotaktischen Polypropylen-Homopolymer mit einem isotaktischen Index von 90 bis 99 % erhalten wird und zwei endotherme Differentialscanningkalorimeter (DSK)-Peaks zwischen 155 und 170°C zeigt, wobei die Faser einen Schmelzindex (Ml_{c}) von 16,5 bis 80,0 und einen Polydispersitätsindex (Pl_{c}) von 2,1 bis 5,7 aufweist.

2. Polypropylen-Faser nach Anspruch 1, bei der die beiden endothermen Differentialscanningkalorimeter (DSK)-Peaks aus einem ersten, bei 160 ± 3 °C erscheinenden endothermen Peak und einem zweiten, bei 165 ± 3 °C erscheinenden endothermen Peak zusammengesetzt sind.

3. Polypropylen-Faser nach Anspruch 1, bei der die Faser einen Schmelzindex (Ml_{c}) von 16,5-80,0 aufweist.

4. Polypropylen-Faser nach Anspruch 1, bei der die Faser einen Polydispersitätsindex (Pl_{c}) von 2,1-5,7 aufweist.

5. Polypropylen-Faser nach Anspruch 1, bei der die Faser eine Feinheit von 1,0-80,0 Denier pro Filament aufweist.

6. Polypropylen-Faser nach Anspruch 4, bei der die Faser einen Pl_{c} von 2,3-4,5 aufweist.

7. Polypropylen-Faser nach Anspruch 1, weiter umfassend einen Stabilisator und/oder ein Antioxidans in einer Menge von 0,03 bis 2,0 Gew.-%.

8. Polypropylen-Faser nach Anspruch 7, bei der der Stabilisator und/oder das Antioxidans in einer Menge von 0,03 bis 0,7 Gew.-% enthalten ist.

9. Polypropylen-Faser nach Anspruch 8, bei der der Stabilisator und/oder das Antioxidans in einer Menge von 0,03 bis 0,4 Gew.-% enthalten ist.

10. Verfahren zur Herstellung von Polypropylen-Fasern, umfassend die Schritte:
(a) Schmelzen eines isotaktischen Polypropylen-Homopolymers mit einem isotaktischen Index von 90-99 %, einem Schmelzindex (Mlₐ) von 10,0-40,0 und einen Polydispersitätsindex (Plₐ) von 2,5-6,0 in einem Extruder, um ein geschmolzenes Polymer zu ergeben, das einen Schmelzindex (Ml_{b}) mit einem Verhältnis von Ml_{b}/Mlₐ im Bereich von 1,01 bis 1,50 und einen Polydispersitätsindex (Pl_{b}) von enger als 10 % oder weniger als der Plₐ aufweist;
(b) Spinnen des geschmolzenen Polymers und Steuern der Quench-Bedingung nach dem Spinnen, um Fasern mit einem Schmelzindex (Ml_{c}) von 16,5-80,0 und einem Polydispersitätsindex (Pl_{c}) zu bilden, der um 20 % oder weniger als der PIₐ enger ist, wobei das Verhältnis von MI_{c}/MIₐ im Bereich von 1,65 bis 7,50 liegt; und
(c) gegebenenfalls Strecken der Fasern.

11. Verfahren nach Anspruch 10, in dem das Polypropylen-Homopolymer einen Stabilisator und/oder ein Antioxidans in einer Menge von 0,03-2,0 Gew.-% in Schritt (a) enthält.

12. Verfahren nach Anspruch 10, in dem der Mlₐ im Bereich von 10 bis 30 liegt.

13. Verfahren nach Anspruch 10, in dem der Plₐ im Bereich von 2,8 bis 5,0 liegt.

14. Verfahren nach Anspruch 13, in dem der Plₐ im Bereich von 3,5 bis 4,3 liegt.

15. Verfahren nach Anspruch 10, in dem die Feinheit der Fasern im Bereich von 1,0 bis 80,0 Denier pro Filament liegt.

16. Verfahren nach Anspruch 10, in dem der MI_{b} im Bereich von 10,1-41,0 liegt.

17. Verfahren nach Anspruch 10, in dem die Faser einen Pl_{c} von 2,1-5,7 aufweist.

18. Verfahren nach Anspruch 17, in dem die Faser einen Pl_{c} von 2,3-4,5 aufweist.
